

## UNITED STATES PATENT OFFICE

1,944,179

## FERROUS ALLOY

Victor O. Homerberg, Belmont, Mass., assignor  
to The Nitromal Corporation, Albany, N. Y.,  
a corporation of Delaware

No Drawing. Application May 10, 1929  
Serial No. 362,136

2 Claims. (Cl. 148—31)

My invention relates to ferrous alloys and particularly to white, mottled and malleable cast irons containing elements rendering them amenable to surface hardening by the nitriding process.

5 While it has been proposed to harden ordinary gray cast iron or steel by subjecting it to the action of ammonia at a temperature of from 900 to 1800 degrees Fahrenheit, experimental work along this line has indicated the impossibility of 10 obtaining a product which, from a practical or commercial viewpoint, is satisfactory.

No appreciable hardening can be attained by nitriding ordinary cast iron at a temperature as low as 900 degrees F., nor can such iron be hardened to an appreciable degree by nitriding at temperatures as high as 1800 degrees F., without additional heat treatment. Furthermore, the case produced in either instance is brittle and susceptible to spalling and exfoliation.

15 It has also been proposed to harden gray cast iron alloys by the Fry nitriding process thereby attaining a final hardness said to correspond to that of hard chill castings or, in other words, to the hardness of white cast iron, to which this invention more particularly relates.

20 White cast iron is very difficult or almost impossible to machine but can be malleableized and is adapted for many uses for which gray cast iron is wholly unsuited. When malleableized it 25 may be machined, and if, thereafter, the surface portions subjected to wear can be appreciably hardened the field of application will be enormously extended.

In order to appreciably harden steel by nitriding, certain alloying elements, such as aluminum for example, and preferably other elements also, must be incorporated therein. It is not apparent that the addition to white cast iron of an alloying element or elements essential to nitriding

will not prevent the malleableizing of the iron, nor is it apparent that after malleableizing such a white cast iron alloy it can be again hardened by nitriding to a degree sufficient to make a commercially desirable product.

60 I find, however, that the addition of small quantities of aluminum, say from 0.15% to 5.0% to a white cast iron having a total carbon content of from about 2.0% to 4.5% produces an alloy which can be malleableized and, moreover, can 65 be satisfactorily nitride hardened at comparatively low temperatures.

To avoid warping and distortion in treating such a malleableized cast iron by the nitriding process it is extremely important that the operation be conducted at a temperature which is not in excess of the thermal critical point (Ac<sub>1</sub> point) of the alloy.

70 While I have mentioned only aluminum as an essential alloy ingredient, it is to be understood that other elements such as boron, chromium, copper, manganese, molybdenum, nickel, silicon, titanium, tungsten, zirconium or vanadium may be present in a combined total amount up to about 8.0% without departing from the true scope and spirit of my invention.

75 What I claim is—

1. An article of manufacture composed of malleableized cast iron having nitride hardened surface portions and containing more than 0.15% 80 and less than 5% of aluminum as an essential alloying ingredient.

2. An article of manufacture composed of malleableized cast iron having nitride hardened surface portions and containing more than 0.15% 85 and less than 2% of aluminum as an essential alloying ingredient.

VICTOR O. HOMERBERG.

95

100

90

105

95

110

**CERTIFICATE OF CORRECTION.**

**Patent No. 1,944,179.**

**January 23, 1934.**

**VICTOR O. HOMERBERG.**

**It is hereby certified that error appears in the printed specification of the above numbered patent requiring correction as follows: Page 1, line 91, claim 2, for the words "and less than" read but not over; and that the said Letters Patent should be read with this correction therein that the same may conform to the record of the case in the Patent Office.**

**Signed and sealed this 13th day of November, A. D. 1934.**

**Leslie Frazer**

**(Seal)**

**Acting Commissioner of Patents.**